

# UNITED STATES PATENT OFFICE.

DAVID GESTETNER, OF TOTTENHAM HALE, ENGLAND.

## PREPARATION AND TREATMENT OF STENCIL-PAPER.

1,125,835.

Specification of Letters Patent.

Patented Jan. 19, 1915.

20 Drawing.

Application filed November 9, 1908. Serial No. 461,801.

To all whom it may concern:

Be it known that I, DAVID GESTETNER, a subject of the King of Great Britain, residing at Tottenham Hale, in the county of Middlesex, England, have invented new and useful Improvements in the Preparation and Treatment of Stencil-Paper, of which the following is a specification.

This invention relates to improvements in the preparation and treatment of stencil paper with a view to the waxy composition used in its preparation being maintained in a soft condition until the stencil is written and then becoming hard or dry and tough in a short time to enable it to resist the action of the ink and the mechanical action of the printing process. For this purpose I employ in the preparation of stencil paper a waxy composition consisting preferably of 20 Java paraffin wax or carnauba wax or a mixture of the two in combination with linseed oil or with the fatty acids of linseed oil. Instead, however, of using the above mentioned waxes and oil or fatty acids, other 25 waxes, drying oil or fatty acids of a drying oil may be employed.

The materials may be combined in the following proportions which I have found to answer well, but other widely different proportions may be used with more or less satisfactory result.

### By weight.

|                                                             |          |
|-------------------------------------------------------------|----------|
| Paraffin wax preferably of the                              |          |
| Java variety                                                | 3 parts. |
| Fine quality of carnauba wax                                | 1 part.  |
| Linseed or other drying oil or a fatty acid of a drying oil | 3 parts. |

In order that the wax employed may resist attack from the oily ink generally used in printing from stencils, it should be of high quality quite free from the wax oils and soft waxes. When using carnauba wax it should be of the fatty variety freed from earthy matter and other impurities. When using linseed oil acids, they are prepared preferably from tanked oil that has been well matured and that is quite free from added impurities. This oil should be treated with caustic soda in quantity insufficient to completely saponify it. The soapy matter thus formed is broken up with dilute mineral acids. The fatty acids thus liberated are washed free from mineral acids and glycerin, thus producing linseed oil acids of

suitable character. Adulterated linseed oil, which frequently contains cotton seed and other oil, will not give good results.

The materials used are melted together and well stirred, care being taken to avoid excessive heat, heat just sufficient to melt them and enable them to be well mixed being that found most suitable. The composition thus prepared is spread on yoshino or like paper in the usual manner. Stencil paper thus prepared is then packed in a container and preferably in the form of a roll, which container then has the air exhausted as far as possible from it and is provided with a cover held in close contact with its seat by atmospheric pressure.

It is preferable to place a few drops of turpentine or other volatile material inside the container, which, when the latter is exhausted will give off a vapor which prevents or delays the hardening of the waxy composition. The container may, however, after exhaustion, be filled with an inert gas.

The ink employed for use with stencils prepared as above should not contain any ingredient prejudicial to the waxy composition, such for instance as glycerin, a drying oil or mineral oils.

Stencil paper having a waxy composition of the character above described spread thereon has the following properties:—The waxy composition is soft and easily removed from the paper by the act of writing a stencil and it can be kept in soft condition for considerable periods when inclosed in a case from which the air is exhausted and which may contain vapor of volatile material or an inert gas. On removal of the stencil paper from its container and on exposure to the air the waxy composition hardens quickly and the hardening is not appreciably delayed by contact with ink if the latter is of suitable character as above explained nor is it affected by continuous contact with such ink under any climatic condition.

What I claim is:—

1. A stencil-paper coated with a composition comprising pure paraffin wax, and linseed oil in proper proportion to be and remain soft when air is excluded therefrom, and for a sufficient time after exposure to air to permit characters to be formed therein by pressing type against the same, and to harden and become dry and tough.

with comparative rapidity upon exposure to the air, substantially as set forth.

2. A stencil-paper coated with a composition consisting of soft paraffin wax, carnauba wax and a rapidly oxidizing material, substantially as set forth.

3. A stencil-paper coated with a composition comprising a wax-like material and a rapidly oxidizing material, said composition being characterized by the properties of remaining soft when air is excluded therefrom and for a sufficient time after exposure to air to permit characters to be formed thereon by pressing smooth-faced type against the same, of being non-adhesive, and of hardening on exposure to air thereafter, substantially as set forth.

4. The process of preparing a stencil, which comprises providing a fibrous base with a coating composition which remains soft out of the presence of air and for a short time after exposure to air, and subsequently hardens on exposure to air, such composition comprising a wax-like material and an oxidizing material, forming characters thereon before said coating has hardened, and then permitting the same to

harden by sufficient exposure to the air, substantially as set forth.

5. The process of manufacturing a stencil, which comprises providing a fibrous base with a coating composition which remains soft out of the presence of air and for a short time after exposure to air, and subsequently hardens on exposure to air, such composition comprising a wax-like material and an oxidizing material, keeping the stencil out of the presence of atmospheric air from the time said soft coating is applied to the base until occasion for forming characters thereon has substantially arrived, then forming characters on said coating, by pressing type or the like against the same, before said coating has hardened, and then permitting said coating to harden by sufficient exposure to the air, substantially as set forth.

In witness whereof I have hereunto set my hand in presence of two witnesses.

DAVID GESTETNER.

Witnesses:

HENRY HASPER,  
WOLDEMAR HAUPT.